

July 21, 1942.

R. L. WORMELL

2,290,789

MANUFACTURE AND PRODUCTION OF ARTIFICIAL  
FILAMENTS, THREADS, AND THE LIKE  
Filed Nov. 14, 1938



INVENTOR

ROBERT LOUIS WORMELL

BY  
*Harrison and Stover*

ATTORNEYS

## UNITED STATES PATENT OFFICE

2,290,789

## MANUFACTURE AND PRODUCTION OF ARTIFICIAL FILAMENTS, THREADS, AND THE LIKE

Robert Louis Wormell, Coventry, England, assignor to Courtaulds, Limited, London, England, a British company

Application November 14, 1938, Serial No. 240,427  
In Great Britain November 18, 1937

## 1 Claim. (Cl. 18—54)

This invention relates to the manufacture and production of threads and the like from casein, or protein compounds having similar properties. Within the term "threads and the like" I wish to include filaments, fibres, yarns and threads of any denier or cross-sectional shape and bands or tows consisting of any number of such filamentary articles. They may be produced, for example, by extruding a solution of a protein through one or more jets each provided with one or more holes and setting the extruded material in any known manner. Each jet may extrude one or a plurality of filaments. If more than one filament is extruded from a jet they are usually formed into a single thread. Any desired number of jets may be used and if desired all the resulting filaments may be brought together to form a tow or band of very considerable denier. It has already been proposed to produce a thread by extruding a solution of casein or the like material through a jet provided with one or more holes into a coagulating bath and subjecting the resulting thread to a treatment, which we will hereinafter refer to as "hardening," which comprises passing the thread through one or more aqueous solutions of substances such as formaldehyde and, aluminium salts, and which renders the thread more resistant to the disintegrating, dissolving or swelling action of water or aqueous solutions and improves the properties of the thread finally obtained. A process is also already known wherein casein fibres are drawn with a speed which is higher, for example 50 per cent higher, than that of spinning and are conveyed under tension through one or more baths of such hardening agents.

According to the present invention the process for improving the properties of threads and the like produced from casein or the like protein substances and hardened, comprises stretching them and thereafter treating them with a hardening agent without allowing them to contract.

The threads may have been produced from casein in any known manner and besides having been subjected to a hardening treatment may have been subjected to any other desired treatments such as washing, stretching or heating before arriving at the stage at which the process of the present invention is applied.

The process of the present invention may be carried out as a continuation of the process of manufacturing the threads or it may be carried out some time afterwards. It is very desirable in both cases to effect the stretching in the presence of a wetting agent, for example water or

an aqueous solution. Aqueous solutions of the lower fatty acids are particularly suitable, and the same solution as that used for hardening may also be used. Stretching should preferably be sufficient to effect an appreciable reduction in the denier of the thread and may be for example, between 50 and 200 per cent. It may be carried out by passing the thread over two or more rotating rollers the second and succeeding ones of which are rotated with peripheral speeds greater than that of the first.

Treatment with the hardening agent may be effected by passing the thread through an atmosphere containing a hardening agent, for example, formaldehyde in vapour form. It may also be effected by passing the thread through a solution containing one or more hardening agents, as for example natural or synthetic tanning agents, formaldehyde or aluminium salts which may be normal or basic salts.

A suitable solution has the following composition:

|                   | Parts |
|-------------------|-------|
| Aluminium acetate | 10    |
| Formaldehyde      | 10    |
| Water             | 80    |

Other substances may also be added to the hardening bath for other purposes, for example, acetone or alcohol for lowering the specific gravity thereof, or salts such as calcium chloride or sodium sulphate for preventing swelling of the threads.

The treatment with a hardening agent after the stretching may or may not result in the complete insolubilisation of the threads, but in any case must be sufficient to minimise considerably the contraction of the stretched threads when released from tension. If insolubilisation is not complete after leaving the said hardening bath it may be completed at a later stage as desired.

The threads may be dried while in the stretched condition before passing to the said treatment with the hardening agent.

The threads may be prevented from contracting after stretching by maintaining the stretched condition by mechanical means; for example the threads may be drawn through the hardening bath at the same speed as they leave the stretching device, or they may be simply wound on reels or bobbins after they have been saturated with hardening liquid. Alternatively contraction may be largely prevented by carrying out the hardening treatment in the presence of

a salt or salts such, for example, as calcium chloride or sodium sulphate.

The threads after treatment according to the present invention may be collected in the form, for example, of a cake or bobbin, or they may be cut into staple fibres. In the latter case, cutting may take place either after complete hardening, washing and drying of the threads, or immediately after they have left the hardening bath in which case the cut threads may need to be left in the wet state for a suitable period until hardening is completed, after which they can be finally washed and dried.

The following example illustrates one method of carrying out the present invention although the invention is not restricted to this example.

*Example*

Casein threads of denier 2400 containing 600 filaments are drawn off by godets from a coagulating bath containing salts and acid. The threads are passed for 15 minutes through a hardening bath consisting of 10 per cent aluminium acetate solution and 10 per cent formaldehyde. The yarn on leaving this apparatus is then passed through a bath of 20 per cent formic acid, in which it is stretched 100 per cent by means of conical godets grooved in steps. Thereafter, while still under tension, it passes through another bath containing the 10 per cent aluminium acetate—10 per cent formaldehyde mixture, and is then wound up on a drum. The yarn after being left on the drum for 15 minutes is cut off and immersed in a bath containing formaldehyde, sodium sulphate and aluminium sulphate at 25° centigrade for 24 hours. It is subsequently immersed in the same mixture at 45° centigrade for 48 hours and is thereafter washed thoroughly in water and dried.

The drawing illustrates in diagrammatic form apparatus suitable for carrying the invention into effect although the invention is not restricted to the form of apparatus shown.

5 Casein solution is extruded through a nozzle 1 into a bath of coagulant 2 and the resulting thread 3 is passed over the guide 4 round rollers 5 and 6 which are rotating at equal speeds and are partially immersed in a bath containing hardening liquid 7. On leaving the roller 6 the thread 10 is passed two or three times round a roller 8 and thence to the roller 9. After passing two to three times round the roller 9 it is passed round the rollers 10 and 11 to a collecting reel 15 12. Roller 8 rotates at substantially the same speed as 5 and 6 and roller 9 at a considerably greater speed while rollers 10 and 11, which are partly immersed in a bath containing hardening liquid 13, both rotate at substantially the same speed as the roller 9. In this case after leaving the coagulating bath the thread is subjected to a hardening treatment without stretching in the bath 7. It is then stretched between the rollers 8 and 9 and is then finally hardened without stretching in the bath 13.

What I claim is:

A process for the manufacture and production of threads and the like, which comprises extruding a solution containing casein into a coagulating medium, drawing off filaments from said coagulating medium and subjecting them to a preliminary hardening treatment, and thereafter improving the properties of the thread by stretching them and then subjecting them to a second hardening treatment without allowing them to contract.

ROBERT LOUIS WORMELL.